

## UNITED STATES PATENT OFFICE

2,163,146

## TAURIDES

Karl Kumetat, Wolfen, Bitterfeld, and Sebastian Gassner, Leverkusen, near Cologne, Germany, assignors, by mesne assignments, to Agfa Anasco Corporation, Binghamton, N. Y., a corporation of Delaware

No Drawing. Original application October 7, 1936, Serial No. 104,442, Patent No. 2,131,742. Divided and this application September 18, 1937, Serial No. 164,500. In Germany October 11, 1935

5 Claims. (Cl. 260—371)

Our present invention relates to taurides. This application is a division of our application Ser. No. 104,442, filed October 7, 1936, now Patent No. 2,131,742.

One of its objects is to provide a tauride of a compound selected from the group consisting of anthraquinone carboxylic acids and anthraquinone sulfonic acids. Another object are new desensitizers. Further objects will be seen from the detailed specification following hereafter.

It has been proposed to use water-soluble derivatives of anthraquinone or phenanthrenequinone, particularly anthraquinone carboxylic acids and anthraquinone sulfonic acids for desensitizing light-sensitive, particularly panchromatic, silver halide emulsions. These water-soluble compounds, however, have not come into use because their desensitizing effect is comparatively small and is considerably inferior to that of the known pinacrytol green. Some of the said compounds are also open to the objection that they form precipitates in water containing lime compounds, and others that they are colored. Both of these properties are undesirable in a desensitizer.

This invention is based on the observation that the taurides of anthraquinone-carboxylic acids and sulfonic acids have a pronounced desensitizing capacity and are free from the foregoing objections. Their desensitizing effect exceeds considerably that of the hitherto known best desensitizer, namely pinacrytol green. The taurides do not form sparingly soluble lime salts and are colorless. Owing to the combination of these favorable properties, the taurides may be regarded as ideal desensitizers. They may be used either in a preliminary bath or as an addition to the developer. Where a preliminary bath is used its desensitizing effect may be considerably enhanced by addition of sodium sulfite. Correspondingly when used in the developer their effect is the stronger the more sodium sulfite the developer contains. Suitable compounds are for instance anthraquinone-sulfotauride, anthraquinone-1-sulfomethyl-tauride, anthraquinone-2-sulfomethyltauride, anthraquinone-2-chloro-3-sulfomethyl-tauride, anthraquinone-2, 6-disulfomethyl-tauride, anthraquinone-2-carbonylmethyltauride and anthraquinone-2-chloro-3-carbonyl-methyltauride.

The following examples illustrate the invention:

1. 1 gram of the sodium salt of anthraquinone-1-sulfomethyltauride is dissolved in 1 litre of water and in this solution orthochromatic or panchromatic photographic layers are bathed for 2

minutes. Development may then follow, for example in a bright green light. The methyltauride salt may be produced as follows (parts being by weight):

To 30 parts of anthraquinone-1-sulfochloride (obtainable by condensing potassium anthraquinone-1-sulfonate with phosphorus pentachloride) mixed with 300 parts of water there are added 30 parts of methyltaurine. The whole is heated at about 80° C. with stirring until the chloride is completely dissolved, and filtered if necessary. To the solution sodium chloride is added whereby the sodium salt of anthraquinone-1-sulfo-methyltauride is precipitated.

2. 1 gram of the sodium salt of anthraquinone-1-sulfo-methyltauride obtained in an analogous manner to that described in Example 1, the parent material being anthraquinone-2-sulfochloride, is dissolved in 1 litre of water, together with 25 grams of anhydrous sodium sulfite. In this solution photographic layers are bathed for 2 minutes and may then be developed in a bright green light.

3. Orthochromatic and panchromatic photographic layers are developed in one litre of a developer of the following composition:

|                                                        |       |     |
|--------------------------------------------------------|-------|-----|
| Water                                                  | litre | 1   |
| Metol (mono-methyl-p-aminophenol)                      | grams | 8   |
| Anhydrous sodium sulfite                               | do    | 125 |
| Anhydrous sodium carbonate                             | do    | 5.8 |
| Potassium bromide                                      | do    | 2.5 |
| The sodium salt of anthraquinone-2-sulfo-methyltauride | do    | 0.5 |

The development may be first for 1 minute in the dark and then continued in a bright green or yellow light.

The simplest compounds of the class of substances to which the invention relates may be represented by the following formulae:

(a) Anthraquinone-2-sulfotauride



(b) Anthraquinone-2-carbonyltauride



## (c) Anthraquinone-2-sulfomethyltauride



## 10 (d) Anthraquinone-2-carbonylmethyltauride



## 20 (e) Anthraquinone-2-chloro-3-sulfomethyltauride



The above named five compounds may be obtained in a manner analogous to that described in Example 1. The components of reaction are in example—

(a) Anthraquinone-2-sulfochloride and taurine;

(b) Anthraquinone-2-carbonylchloride and taurine;

(c) Anthraquinone-2-sulfochloride and methyltaurine;

(d) Anthraquinone-2-carbonylchloride and methyltaurine; and

40 (e) Anthraquinone-2-chloro-3-sulfochloride and methyltaurine.

What we claim is:

1. A tauride of a compound selected from the group consisting of anthraquinone carboxylic acids, anthraquinone sulfonic acids and such

acids in which the nucleus is substituted by halogen.

2. An anthraquinone tauride corresponding with the general formula



X stands for a member of the group consisting of CO and SO<sub>2</sub>; Y stands for a member of the group consisting of H and alkyl.

3. Anthraquinone-2-carbonylmethyltauride corresponding with the formula



4. Anthraquinone-2-sulfomethyltauride corresponding with the formula



5. Anthraquinone-2-chloro-3-sulfomethyltauride corresponding with the formula



KARL KUMETAT.

SEBASTIAN GASSNER.

45